

## 1

3,576,592

### PROCESS FOR PERMANENTLY PRESSING TEXTILE ARTICLES MADE OF KERATINIC FIBERS

Charles Zviak, Franconville, and Andre Viout, Paris, France, assignors to Societe Anonyme dite: L'Oreal  
No Drawing. Filed Feb. 21, 1966, Ser. No. 528,762  
Claims priority, application France, Feb. 23, 1965,  
6,590; Aug. 5, 1965, 27,374  
Int. Cl. C09k 3/30; D06m 15/12

U.S. Cl. 8—127.6

2 Claims

#### ABSTRACT OF THE DISCLOSURE

The method of permanently pressing textile articles containing keratinic fibers, which comprises the steps of impregnating the textile article with a solution containing effective amounts of a water soluble polymer having branched chains having terminal —SH functional groups, placing the impregnated textile article in the configuration corresponding to the shape desired, and then pressing the area in which a crease is desired at an elevated temperature.

It is known that it is desirable to impress creases in the most durable manner possible on textile articles, for example, creases in pants or in pleated skirts.

The present invention relates to a new process for permanently pressing cloth or knitted materials made of wool, so that it will be resistant to wrinkles and permanently retain creases made therein at the time of treatment.

These creases may be obtained according to the invention in a simple and durable manner without causing damage to or weakening of the physical properties of the textile articles.

One object of the present invention is to present a new process for making creases in textile articles made of keratinic fibers, this new process being characterized by the fact that the above-mentioned textile articles are impregnated with a basic solution of polysulphydrylated polymers, then heated and pressed in the area in which a crease is desired, for example, by using an iron.

According to the invention, the solution to be applied to the textile article contains about 1 to 20% and preferably from 2 to 6% by weight of polysulphydrylated polymers.

The pH of this solution is between about 3.5 and 10 and is preferably between 9 and 9.5.

Among the polysulphydrylated polymers which can be used to carry out the process according to the invention, are the polysulphydrylated polymers corresponding to the following formula:



in which:

R<sub>1</sub> is an alkyl radical comprising preferably from 2 to 4 carbon atoms, which may be substituted by lower alkyls having up to 4 carbon atoms, by a carboxyl radical or by a carbalkyloxy group,

R is a hydrogen atom or a lower alkyl such as —CH<sub>3</sub> or —C<sub>2</sub>H<sub>5</sub>,

R' and R'' are hydrogen atoms, lower alkyl radicals, phenyl radicals or lower alkylloxy radicals, R' and R'' being the same or different, R''' being a hydrogen atom,

## 2

or a —OCOCH<sub>3</sub> radical, or a —COOCH<sub>3</sub> radical, or a —CN radical,  
n is a whole number.

The polysulphydrylated polymers are of the formula:



in which:

20 R<sub>1</sub> is a hydrogen atom or a lower alkyl such as CH<sub>3</sub> or C<sub>2</sub>H<sub>5</sub> or a lower hydroxy alkyl such as —CH<sub>2</sub>CH<sub>2</sub>—OH

R<sub>2</sub> is a hydrogen atom or a —CH<sub>3</sub> radical,

25 q is a whole number between 2 and 6, inclusive,  
p is a whole number equal to 0 or 1,  
R' and R'' are hydrogen atoms or lower alkyl radicals, or phenyl radicals, or lower alkylloxy radicals, R' and R'' being the same or different,

30 R''' is a hydrogen atom, or the —OCOCH<sub>3</sub> radical, or the —C≡N radical, or the —COOCH<sub>3</sub> radical,  
n is a whole number.

The polysulphydrylated polymers are of the formula:



40 in which:

R' and R'' which may be the same or different are hydrogen atoms, or lower alkyl radicals, or phenyl radicals, or lower alkylloxy radicals,

45 R''' is a hydrogen atom, or the —OCOCH<sub>3</sub> radical, or the —COOCH<sub>3</sub> radical, or the —C≡N radical,  
n is a whole number,  
Q is a radical represented by the following formula:



50 in which:

R<sub>1</sub> is H or CH<sub>3</sub>,

R<sub>2</sub> is H or COOH,

q is a whole number from 1 to 5, inclusive,

55 q' is equal to 0 or 1,

p is equal to 0 or 1,

Q' is a radical represented by the following formula:



60 in which:

R<sub>2</sub> is a hydrogen atom or a lower alkyl,  
R<sub>4</sub> is a lower alkyl, or a radical or formula



65 r and r' being the same or different lower alkyls, or being part of a heterocyclic ring such as that of morpholine or piperidine, m is a whole number equal to 2, 3 or 4.

The polysulphydrylated polymers are constituted by an anhydride homopolymer on which at least one mercapto-amine is condensed.

The homopolymer may be a maleic polyanhydride polymer, an itaconic polyanhydride polymer, an acrylic polyanhydride polymer, a mixed acrylic-methacrylic polyanhydride polymer, or a methacrylic polymer, although this list is not exhaustive.

Aminothiols having the following formula may be used to sulphydrylate these homopolymers:



in which:

R is an alkylene radical comprising preferably from 2 to 4 carbon atoms, which may be substituted by lower alkyls which may have up to 4 carbon atoms, or a carboxyl radical, or a carbalkyloxy group, and R' is a hydrogen atom or a lower alkyl such as  $-\text{CH}_3$  or  $-\text{C}_2\text{H}_5$ .

Among the aminothiols corresponding to the above formula, these may be cited as examples:

$\beta$ -mercaptoproethylamine,  
cysteine, and  
ethyl cysteinate.

Mercapto-amide amines of the following formula may also be used to sulphydrylate the homopolymers:



in which:

R<sub>1</sub> is H,  $-\text{CH}_3$ ,  $-\text{C}_2\text{H}_5$ , or  $-\text{CH}_2-\text{CH}_2-\text{OH}$ , R<sub>2</sub> is H or  $-\text{COOH}$ , q is a whole number between 1 and 5, inclusive, q' is equal to 0 or 1, p is equal to 0 or 1.

Among the mercapto-amide amines corresponding to this last formula may be cited those which are obtained from esters of thioglycolic acid, thiolic acid or  $\beta$ -mercaptopropionic acid and from diamines such as ethylene diamine, hexamethylene diamine, N-hydroxyethyl ethylene diamine.

It is equally possible to condense amines not made up of  $-\text{SH}$  groups on the anhydride homopolymers, with simultaneous condensation of the mercapto-amines.

Another object of the present invention is to provide a new article of manufacture which consists of a composition for permanently creasing textile articles made from keratinic fibers. This composition is essentially characterized by the fact that it contains at least one polysulphydrylated polymer and a base, the pH of this composition being between about 3.5 and 10 and being preferably between 9 and 9.5.

In a preferred method of treating with aforementioned composition this last is placed in an aerosol bomb with a liquified gas propellant under pressure, from which it is permitted to escape as a lather or a jet of liquid which may be atomized.

In order that the invention may be better understood, several embodiments thereof will now be described, purely by way of example, without limiting the scope of the invention to the specific details thereof.

#### EXAMPLE I

A composition may be made according to the invention by mixing:

A polysulphydrylated polymer obtained by reacting  $\beta$ -mercaptoproethylamine with the styrene/maleic anhydride copolymer sold by the Texas Butadiene Chemical Corp.

5  
10

under the trademark "Resin SMA 1000A" having the formula:



De-ionized water—959 g.  
Monethanol to bring the pH of the solution to 9.5 about 11 g.

15  
20  
25  
30

The woolen cloth in which a permanent crease is desired is dampened with this solution; then the cloth is ironed to impress the crease using a hot iron and a damp cloth.

When the cloth has dried and cooled off, it has a permanent crease which remains even after several washings.

#### EXAMPLE 2

A composition to obtain permanent creases in textile articles of keratinic fibers is prepared as follows:

First solution A having the following composition is prepared:

|                                                                    |       |    |     |
|--------------------------------------------------------------------|-------|----|-----|
| A polysulphydrylated polymer as in Example 1 above                 | ----- | g  | 40  |
| 30 Ammonia at 20 Bé. to bring the pH of the solution to 9.5, about | ----- | cc | 60  |
| De-ionized water                                                   | ----- | g  | 900 |

The following mixture is then placed in an aerosol container:

|    |                            |       |    |    |
|----|----------------------------|-------|----|----|
| 35 | Solution A                 | ----- | G. | 70 |
|    | Dichlorodifluoromethane    | ----- |    | 15 |
|    | Trichloromonofluoromethane | ----- |    | 15 |

40  
45  
50

To use the composition, which is in the form of an aerosol, the solution contained in the bomb is sprayed onto the textile article to be creased, then a crease is formed using a hot iron and a damp cloth.

#### EXAMPLE 3

To prepare a composition according to the invention in the form of a transient lather spread by an aerosol bomb, the following process is used:

First solution B having the following composition is prepared:

|                                                     |       |    |     |
|-----------------------------------------------------|-------|----|-----|
| A polysulphydrylated polymer as in Example 1 above  | ----- | g  | 30  |
| 55 De-ionized water                                 | ----- | g  | 920 |
| 55 Ammonia at 20° Bé. to bring the pH to 9.5, about | ----- | cc | 45  |
| Silicone anti-foaming agent                         | ----- | g  | 4   |
| Polyethoxyether of a fatty alcohol                  | ----- | g  | 1   |

60  
65  
70

After this a mixture consisting of the following is placed in a special container:

|            |                         |       |    |    |
|------------|-------------------------|-------|----|----|
| Solution B | -----                   | G.    | 85 |    |
|            | Dichlorodifluoromethane | ----- |    | 15 |

65  
70  
75  
80

The aerosol container has an atomizing valve which permits a ribbon of lather to be put on the cloth to be treated around the crease. The latter disappears rapidly, impregnating the underlying cloth with the composition according to the invention.

As in the preceding examples, a crease of excellent quality is obtained using a hot iron and a damp cloth.

This method of treating with the composition according to the invention has the advantage of being very practical in use and of avoiding the oxidation of the polysulphydrylated polymer.

5  
EXAMPLE 4

A composition according to the invention is obtained by mixing:

A polysulfhydrylated polymer obtained by condensation of a mol of  $\beta$ -mercaptoethylamine on a mol of maleic anhydride/ethylene copolymer sold by the Monsanto Corp. under the trademark "Resin DX 840.11" having the formula:



Ammonia at 20° Bé. q.s.p. pH=9.3.  
Distilled water q.s.p. 100 cc.

A crease is made in a woolen cloth as in the preceding examples, using a hot iron and a damp cloth.

The permanent press thus obtained holds up well even when the cloth is placed in boiling water for an hour.

6

|                                              |      |     |
|----------------------------------------------|------|-----|
| A polysulfhydrylated polymer as in Example 5 | —g—  | 1.5 |
| Ammonia at 20° Bé. q.s.p. pH 9.3.            |      |     |
| Silicone anti-foaming agent                  | —g—  | 0.4 |
| Water, q.s.p.                                | —cc— | 100 |

5 The following mixture is then put in an aerosol container:

|            |     |    |
|------------|-----|----|
| Solution C | —g— | 85 |
| Butane     | —   | 15 |

10 The contents of the aerosol bomb are sprayed onto the cloth to be treated in the area where pressing is desired. A crease is formed using a hot iron and a damp cloth.

15 Good quality pressing is obtained.

## EXAMPLE 7

A composition according to the invention which is in the form of a transient aerosol lather is made by first preparing a solution D having the following composition:

20 A polysulfhydrylated polymer obtained by condensing  $\beta$ -mercaptoethylamine and N,N-diethyl-propylene diamine on an ethylene/maleic anhydride copolymer having the formula:



## EXAMPLE 5

A solution having the following composition is placed in a roll-on-applicator:

A polysulfhydrylated polymer obtained by condensing a N-( $\beta$ -aminoethyl) thioglycolamide on a ethylene/maleic anhydride copolymer sold under the trademark "Resin DX.840.11" by the Monsanto Chemical Co., this polymer having the formula:



Ammonia at 20° Bé. q.s.p. pH=9.3.  
Distilled water q.s.p. 100 cc.

The cloth to be treated is dampened by rolling the ball of the applicator over the area where pressing is desired, then ironing it with a hot iron.

Thus a crease with excellent holding power is obtained.

## EXAMPLE 6

A composition according to the invention is made in the form of an aerosol by first preparing a solution C having the following composition:

45 Ammonia at 20° Bé. q.s.p. pH 9.3.  
Silicone anti-foaming agent —g— 0.4  
Polyethoxyether of alkylphenol —g— 0.2  
Water, q.s.p. —cc— 100

50 A mixture of the following is then placed in an aerosol bomb:

|                         |     |    |
|-------------------------|-----|----|
| Solution D              | —g— | 85 |
| Dichlorodifluoromethane | —   | 15 |

55 The aerosol bomb has an atomizing valve which permits a ribbon of lather to be placed on the textile article to be treated, in the area of pressing. The lather disappears rapidly, impregnating the cloth below it with liquid.

Pressing is then done as in the preceding example, using a hot iron and a damp cloth and equally good results are obtained.

## EXAMPLE 8

60 A composition is prepared by mixing:  
A polysulfhydrylated polymer obtained by condensing  $\beta$ -mercaptoethylamine and n-butylamine on a vinyl acetate/maleic anhydride copolymer having the formula:



75 Ammonia at 20° Bé. q.s.p. pH=9.3.  
Distilled water, q.s.p. 100 cc.

Woolen cloth is pressed as in the preceding examples, using a hot iron and a damp cloth. The permanent press thus obtained holds up well, even when the cloth is immersed in hot water for an hour.

## EXAMPLE 9

A composition according to the invention is prepared by mixing:

A polysulfhydrylated polymer obtained by condensing N-( $\beta$ -aminoethyl) thioglycolamide on a vinyl acetate/maleic anhydride copolymer having the formula:



Ammonia at 20° Bé. q.s.p. pH=9.3  
Distilled water, q.s.p. 100 cc.

A crease is made in a woolen cloth as in the preceding examples using a hot iron and a damp cloth; the crease thus obtained holds up well even when immersed in hot water for an hour, and remains after several washings.

## EXAMPLE 10

A composition according to the invention is prepared by mixing:

A polysulfhydrylated polymer obtained by condensing  $\beta$ -mercaptoproethylamine on a maleic anhydride/vinyl acetate copolymer having the formula:



Ammonia at 20° Bé. q.s.p. pH=9.3  
Distilled water, q.s.p. 100 cc.

Using the same method as in the preceding examples, a permanent crease is obtained which holds up very well during several washings with very hot water.

## EXAMPLE 11

To obtain a permanent crease in a woolen cloth, a composition according to the invention is prepared by mixing:

A polysulfhydrylated homopolymer having the formula:



De-ionized water 959 g.

Monoethanolamine to bring the pH of the solution to 9.5 about 11 g.

The woolen cloth in which a permanent crease is desired is dampened with this solution. The cloth is ironed with a hot iron and a damp cloth to impress the crease and a permanent crease is obtained which remains even after several washings.

## EXAMPLE 12

A composition to make permanent creases in textile articles made of keratinic fibers is prepared as follows:

First a solution E having the following composition is prepared:

The polysulfhydrylated homopolymer mentioned in Example 11 \_\_\_\_\_ g. 40  
Ammonia at 22° Bé. to bring the pH to 9.5, about \_\_\_\_\_ cc. 65  
De-ionized water, q.s.p. \_\_\_\_\_ g. 1000

The following mixture is then placed in an aerosol bomb:

15 The aforementioned solution E \_\_\_\_\_ 70  
Dichlorodifluoromethane \_\_\_\_\_ 15  
Trichloromonofluoromethane \_\_\_\_\_ 15

To use the composition which is in the form of an aerosol, the solution contained in the bomb is sprayed onto the textile article at the place at which a crease is desired; then the crease is formed using a hot iron and a damp cloth.

## EXAMPLE 13

25 To make a permanent crease in a textile article made of keratinic fibers, a solution having the following composition is placed in a roll-on applicator:

A polysulfhydrylated homopolymer having the formula:



35 Ammonia at 20° Bé. q.s.p. pH=9.3.  
40 Distilled water, q.s.p. \_\_\_\_\_ cc. 100

The cloth to be treated is dampened by rolling the ball of the applicator over the area in which a crease is desired, then ironing with a hot iron.

45 A crease with excellent holding power is thus obtained.

It is clear that the process according to the invention permits the easy and efficient formation of creases in textile articles made of keratinic fibers such as wool.

It should be understood that the above-described embodiments of the invention may be modified as to detail without thereby going outside the scope of the invention.

In particular, it goes without saying that the crease may be formed in the textile article without using a hand iron by using another method such as a pressing machine which permits the simultaneous application of heat and pressure.

It goes equally without saying that the process according to the invention permits the formation of all sorts of creases in textile articles other than woven cloths. In particular, the process according to the invention permits the formation of creases in knitted materials, laces, felts and generally in keratinic textile fibers assembled in any manner whatever.

60 65 70 75 Finally, it is obvious that the process according to the invention is not limited to textile processes carried out using exclusively keratinic fibers such as wool, alpaca, camel's hair or mohair, for treatment according to the invention may be possible even if these keratinic fibers are mixed with other natural, artificial or synthetic textile fibers.

What is claimed is:

1. A process for permanently pressing textile articles containing wool fibers which comprises impregnating the textile with an aqueous solution containing 1-20 weight

percent of a polysulfhydrylated polymer selected from the group consisting of:

(a) water-soluble polysulfhydrylated polymer having recurring units of the formula



5

10

wherein  $\text{R}_1$  is selected from the group consisting of alkylene having 2 to 4 carbon atoms, lower alkyl substituted lower alkylene, carboxy substituted lower alkylene and carbalkoxy substituted lower alkylene,  $\text{R}$  is selected from the group consisting of hydrogen and lower alkyl,  $\text{R}'$  is selected from the group consisting of hydrogen, lower alkyl, phenyl and lower alkoxy,  $\text{R}''$  is selected from the group consisting of hydrogen lower alkyl, phenyl and lower alkoxy and  $\text{R}'''$  is selected from the group consisting of  $-\text{OCOCH}_3$ ,  $-\text{COOCH}_3$  and  $-\text{C}\equiv\text{N}$ ;

(b) a water-soluble polysulfhydrylated polymer having recurring units of the formula



30

35

40

wherein  $\text{R}_1$  is selected from the group consisting of hydrogen, lower alkyl and hydroxy lower alkyl,  $\text{R}_2$  is selected from the group consisting of hydrogen and  $-\text{CH}_3$ ,  $q$  is an integer of 2-6,  $p$  is equal to 0 or 1,  $\text{R}'$  and  $\text{R}''$  are selected from the group consisting of hydrogen, lower alkyl, phenyl and lower alkoxy, and  $\text{R}'''$  is selected from the group consisting of hydrogen,  $-\text{OCOCH}_3$ ,  $-\text{C}\equiv\text{N}$  and  $-\text{COOCH}_3$ ;

(c) a water-soluble polysulfhydrylated polymer having recurring units of the formula



55

wherein  $\text{R}'$  and  $\text{R}''$  are selected from the group consisting of hydrogen, lower alkyl, phenyl and lower alkoxy,  $\text{R}'''$  is selected from the group consisting of hydrogen,  $-\text{OCOCH}_3$ ,  $-\text{COOCH}_3$  and  $-\text{C}\equiv\text{N}$ ,  $\text{Q}$  is a radical of the formula



wherein  $\text{R}_1$  is selected from the group consisting of hydrogen and  $-\text{CH}_3$ ,  $\text{R}_2$  is selected from the group consisting of hydrogen and  $-\text{COOH}$ ,  $q$  is an integer

of 1-5,  $q'$  is equal to 0 or 1 and  $p$  is equal to 0 or 1,  $\text{O}'$  is a radical of the formula



wherein  $\text{R}_3$  is selected from the group consisting of hydrogen and lower alkyl,  $\text{R}_4$  is selected from the group consisting of lower alkyl and



wherein



is selected from the group consisting of lower alkyl amines and a heterocyclic ring selected from the group consisting of morpholino and piperidino rings and  $m$  is an integer of 2-4; and

(d) a water-soluble polysulfhydrylated polymer condensed from (1) an anhydride polymer selected from the group consisting of poly(acrylic anhydride), poly(itaconic anhydride), poly(mixed acrylic-methacrylic anhydride), poly(methacrylic anhydride) and poly(maleic anhydride), and (2) a member selected from the group consisting of

(i) an aminothiol of the formula



wherein  $\text{R}$  is selected from the group consisting of lower alkylene having 2-4 carbon atoms, lower alkyl substituted lower alkylene, carboxy substituted lower alkylene and carbalkoxy substituted lower alkylene and  $\text{R}'$  is lower alkyl and

(ii) a mercapto-amide amine of the formula



wherein  $\text{R}_1$  is selected from the group consisting of hydrogen,  $-\text{CH}_3$ ,  $-\text{C}_2\text{H}_5$  and  $-\text{CH}_2-\text{CH}_2\text{OH}$ ,  $\text{R}_2$  is selected from the group consisting of hydrogen and  $-\text{COOH}$ ,  $q$  is an integer of 1-5,  $q'$  is equal to 0 or 1 and  $p$  is equal to 0 or 1, said solution having a pH ranging from 3.5-10, placing the impregnated textile article in the configuration corresponding to the shape desired and pressing said textile article at an elevated temperature.

2. The process of claim 1 wherein the water-soluble polysulfhydrylated polymer defined in (d) is additionally condensed from (3) a lower alkyl amine.

#### References Cited

##### UNITED STATES PATENTS

- |           |        |                |       |          |
|-----------|--------|----------------|-------|----------|
| 2,238,672 | 4/1941 | Arthur et al.  | ----- | 8-128    |
| 2,933,409 | 4/1960 | Binkley et al. | ----- | 8-128X   |
| 3,148,127 | 9/1964 | Marsh          | ----- | 252-305X |
| 3,247,067 | 4/1966 | Miskel et al.  | ----- | 167-87.1 |

##### FOREIGN PATENTS

- |           |         |        |       |        |
|-----------|---------|--------|-------|--------|
| 1,349,140 | 12/1963 | France | ----- | 260-79 |
|-----------|---------|--------|-------|--------|

65 RICHARD D. LOVERING, Primary Examiner

U.S. Cl. X.R.

8-128; 252-305